

# UNITED STATES PATENT OFFICE.

MARTIN SZAMATOLSKI, OF BAYONNE, NEW JERSEY, ASSIGNEE TO H. BRIDGMAN  
SMITH, OF NEW YORK, N. Y.

## CHROME-LEATHER SOLE FOR BOOTS AND SHOES AND METHOD OF MAKING SAME.

1,173,988.

Specification of Letters Patent. Patented Feb. 29, 1916.

No Drawing.

Application filed May 17, 1913. Serial No. 768,291.

To all whom it may concern:

Be it known that I, MARTIN SZAMATOLSKI, a citizen of the United States, residing at Bayonne, in the county of Hudson and State 5 of New Jersey, have invented new and useful Improvements in Chrome-Leather Soles for Boots and Shoes and Methods of Making Same, of which the following is a specification.

10 My present invention relates to an improved chrome leather sole for boots and shoes, and to an improved method of making or treating the same.

As is well understood by those familiar 15 with the subject, chrome leather in its natural state is not suitable for use as soles in the manufacture of boots and shoes, owing to the fact that this class of leather is naturally soft and loose in fiber, and does not 20 therefore have sufficient firmness or body, or possess proper wearing qualities to warrant its use for the purpose stated, and furthermore in its natural state it is most difficult, if not impossible to properly "edge" 25 the same.

The present invention relates to a leather produced from chrome-leather in such manner as to produce a leather equal in its firmness and wearing qualities to oak-tanned 30 sole leather, and which when used as a sole may readily be edged and one that will be substantially waterproof.

According to the present invention I treat chrome leather, or the soles cut therefrom, 35 with a compound or composition consisting of a resin dissolved in a suitable hydrocarbon solvent, such for instance as naphtha, benzin, or benzol, the latter being preferable, a suitable proportion of any of the known 40 nondrying oils, such as paraffin oil, being added if necessary to give the proper softness and pliability to the finished product.

I may employ resin in any form, such for 45 example as resin or rosin. When rosin is employed it is first ground to a powder and then thoroughly dissolved in the solvent, preferably by stirring or agitating in any suitable way. When sufficiently dissolved the softening oil is added and the mass 50 again thoroughly stirred or agitated. If desired any suitable coloring matter may be added to give the desired color to the finished product.

I have obtained most satisfactory results 55 from a compound consisting of about equal

parts of resin and the solvent, adding from two to ten per cent. of the nondrying oil, although I do not wish to limit myself to the exact proportions stated. Obviously the quantity of oil employed will depend largely 60 upon the softness and flexibility desired to be given to the finished product.

The consistency of the compound is about that of water or perhaps a little thicker, while its natural color will vary from clear 65 to dark amber, although as before stated, any suitable coloring matter may be added.

The compound is comparatively cheap and may be easily and quickly prepared, as will 70 be apparent.

I have discovered that chrome leather and especially sole-blanks stamped or cut from chrome leather to be used in the manufacture of boots, shoes and sandals, when treated with the herein described compound, 75 are at least equal if not superior to oak-tanned sole leather, in firmness and wearing qualities, and not only less expensive, owing to the grade of leather employed, but on account of the ease and rapidity with which 80 the compound may be applied and with which it takes effect.

As is well known by those versed in the art, chrome leather is naturally loose in fiber, soft and otherwise unsuited for use as sole 85 material in the manufacture of boots and shoes, but I have discovered that when treated with the compound herein described the loose fibers become cemented together giving a decided firmness to the leather, 90 equal to that of oak-tanned sole leather and also greatly increasing the wearing qualities and at the same time permitting the sole to be edged, which is a practical impossibility with chrome leather in its natural 95 state, or when treated in any way now known to me.

The chrome leather is treated by immersing the same in the compound, allowing the leather to remain immersed from five seconds to two minutes, depending upon the thickness of the leather. While I prefer the immersion process, I will state that satisfactory results have been secured by applying the compound to the leather with a 100 brush, and also by spraying the compound upon the leather. After the leather has been treated with the compound in either of the ways indicated, it is then allowed to dry, 105 and I have found that complete air drying 110

will take place in from twelve to twenty-four hours. Of course the leather could be dried more quickly if subjected to heat, either in a heated drying room, or otherwise.

An inexpensive and rapid method of treating chrome leather soles according to this invention consists in first cutting out the soles from chrome leather, then placing a number of them in a wire basket and immersing the same in a tank containing the compound, allowing the basket with the soles therein to remain in the compound for a period varying from five seconds to two minutes, depending upon the thickness of the soles. The basket is then withdrawn from the tank, the soles taken out, and dried in any suitable way.

The chief advantages resulting from treating chrome leather soles according to the present invention, reside in the cheapness of the compound, the simplicity of the method,

and the great saving in time and labor over the usual methods of treating leather.

What I claim is:—

1. As a new article of manufacture, a sole for use in the manufacture of boots and shoes, consisting of a chrome leather blank the fibers whereof are impregnated with a compound consisting of substantially five <sup>parts of resin dissolved in substantially five</sup> <sub>parts</sub> <sup>20</sup> parts of naphtha and one part of paraffin oil.

2. A compound for treating leather maintaining a liquid state at ordinary temperatures and consisting of substantially five <sup>35</sup> parts of resin, five parts of naphtha, and one part of paraffin oil.

In testimony whereof I have hereunto set my hand in presence of two subscribing witnesses.

MARTIN SZAMATOLSKI.

Witnesses:

E. H. BICKERTON,  
J. GRANVILLE MEYERS.